

## UNITED STATES PATENT OFFICE

2,356,475

PHENOLIC AND NAPHTHOLIC COUPLERS  
CONTAINING SULPHONAMIDE GROUPSKarl Schinzel, Zurich, Switzerland, assignor to  
Eastman Kodak Company, Rochester, N. Y., a  
corporation of New JerseyNo Drawing. Application March 24, 1939, Serial  
No. 263,945. In Austria July 7, 1936

12 Claims. (Cl. 95—6)

This invention relates to photographic color forming compounds and more particularly to phenolic or naphtholic coupler compounds containing a sulphonamide group.

This application is a continuation in part of my Patent No. 2,306,410, granted December 29, 1942.

The formation of colored photographic images by the use of a primary aromatic amino developing agent, which couples with a color forming compound on development, has been the subject of prior patents. Fischer British Patent 15,055/1912 discloses phenols and naphthols as coupler compounds which are used with p-phenylenediamine couplers. These coupler compounds react with the developing agent during photographic development to form colored photographic images. The dyes formed in this way are insoluble in water and in the ordinary photographic developing and fixing baths although the silver images formed simultaneously with them may be removed from the photographic layer.

Many of the phenolic and naphtholic coupler compounds hitherto used are not sufficiently soluble in the developing solution to enable them to be incorporated in sufficiently large amounts and some of them also tend to produce cloudy or hazy dye images. For these reasons the images obtained do not always have as high dye density as desired and the resulting picture is not clearly transparent.

It is, therefore, an object of the present invention to provide novel photographic coupler compounds having desirable characteristics. A further object is to provide photographic couplers which are highly soluble in developing solutions. A still further object is to provide photographic couplers which produce transparent dyes on photographic development. A still further object is to provide coupler compounds which form dyes of desirable transmission characteristics for multi-color photography.

These objects are accomplished by using as couplers phenolic or naphtholic compounds containing at least one sulphonamide group.

The compounds preferably used as couplers according to my invention are  $\alpha$ -naphthols containing a sulphonamide group ( $-\text{SO}_2\text{NH}_2$ ). The naphthols may contain substituent groups in the rings and the amino group of the sulphonamide substituent may also be substituted at one or both of the hydrogen atoms. Two or more sulphonamide groups may be present in the compound although the position *ortho* or *para* with

respect to the hydroxyl group of the naphthol should preferably be free, or substituted with a replaceable group, since it appears likely that the coupling occurs in one of these positions.

Examples of coupler compounds suitable for use according to my invention are as follows:

15  $\alpha$ -Naphthol-8-sulphonamide $\alpha$ -Naphthol-4-chloro-8-sulphonamide $\alpha$ -Naphthol-3,6-disulphonamide

1-naphthol-8-sulphonanilide



2,4-dichloro-1-naphthol-5-sulphonanilide



1-naphthol-5-sulphonpiperide



N-cyclohexyl-1-naphthol-5-sulphonamide





In place of the  $\alpha$ -naphthols containing a sulphonamide described above, I may also use  $\beta$ -naphthols or phenols. These compounds may contain substituent groups in the ring or rings of the phenolic or naphthoic portion of the molecule as illustrated above or one or both hydrogen atoms of the  $\text{NH}_2$  group of the sulphonamide may be substituted as indicated in the above examples.

The following example, which is illustrative only, indicates a developing solution which may be used according to my invention.

A

|                                      |       |      |    |
|--------------------------------------|-------|------|----|
| Dimethyl-p-phenylenediamine sulphate | grams | 2.5  | 30 |
| Sodium sulphite anhydrous            | do    | 2    |    |
| Sodium carbonate anhydrous           | do    | 20   |    |
| Potassium bromide                    | do    | 1    |    |
| Water to                             | cc.   | 1000 | 35 |

B

|                             |       |     |
|-----------------------------|-------|-----|
| 1-naphthol-5-sulphonanilide | grams | 2   |
| Isopropyl alcohol           | cc.   | 100 |

For use, B is added to A.

In the foregoing examples, I have described adding the coupler compound to the developing solution itself. However, the coupler compound may be incorporated in the photographic layer prior to exposure and the colored image formed by development in the primary aromatic amino developing solution. Special dispersing agents may be used for incorporating the coupler compound in the emulsion and in certain cases the coupler compound may be absorbed or adsorbed to the sensitive salt or may be combined with the sensitive silver salt as a chemical combination. In the case of a multi-layer photographic film in which the color-forming compounds may be incorporated in one or more layers of the film, it may be necessary to take special precautions to prevent wandering of the coupler compound from the sensitive layer in which it is incorporated.

The aromatic amino developing agents used with the coupler compounds of our invention include the mono, di and tri-aminoaryl compounds and their derivatives formed by substitution in the amino group as well as in the ring, such as alkylphenylenediamines and alkyltolylenediamines. These compounds are usually used in the salt form, such as the hydrochloride or the sulphate, which are more stable than the amines themselves. Suitable compounds are diethyl-p-phenylenediamine hydrochloride, monomethyl-p-phenylenediaminehydrochloride, and dimethyl-p-phenylenediaminesulphate. The  $\alpha$ -amino-phenols and their substitution products may also be used where the amino group is unsubstituted. All of these compounds have an unsubstituted

amino group which enables the oxidation products of the developer to couple with the color forming compounds to form a dye image.

My development process may be employed for the products of colored photographic images in layers of gelatin or other carrier, such as collodion, organic esters of cellulose or synthetic resins. The carrier may be supported by a transparent medium such as glass as a cellulose ester or a non-transparent reflecting medium such as paper or an opaque cellulose ester. The emulsion may be coated as a single layer on the support or in the case of a transparent support as superposed layers on one or both sides of the support. The superposed layers may be differentially sensitized and the dyes formed therein by coupling may be bleached by an oxidizing agent such as chromic acid +KBr to colorless soluble compounds. The destruction of the dye in this way does not destroy the silver image and a silver image may be developed, bleached and developed to color a number of times, thus permitting the formation of natural color images and superposed layers as described, for example, in Mannes and Godowsky U. S. Patent No. 2,113,329.

The examples and compounds set forth in the present specification are illustrative only and it is to be understood that my invention is to be taken as limited only by the scope of the appended claims.

I claim:

1. A color-forming photographic developer comprising an aromatic amino developing agent and a coupler compound selected from the group consisting of phenols and naphthols containing at least one sulphonamide group.

2. A color-forming photographic developer comprising an aromatic amino developing agent and a coupler compound comprising an  $\alpha$ -naphthol containing at least one sulphonamide group.

3. A color-forming photographic developer comprising a paraphenylenediamine developing agent and a coupler compound selected from the group consisting of phenols and naphthols containing at least one sulphonamide group.

4. A color-forming photographic developer comprising a paraphenylenediamine developing agent and a coupler compound comprising an  $\alpha$ -naphthol containing at least one sulphonamide group.

5. A color-forming photographic developer comprising an aromatic amino developing agent and a coupler compound comprising  $\alpha$ -naphthol-8-sulphonamide.

6. A color-forming photographic developer comprising an aromatic amino developing agent and a coupler compound comprising  $\alpha$ -naphthol-3:6-disulphonamide.

7. The method of producing a colored photographic image in a gelatino-silver halide emulsion layer, which comprises exposing it and developing it with an aromatic amino developing agent containing a primary amino group in the presence of a coupler compound selected from the group consisting of phenols and naphthols containing at least one sulphonamide group.

8. The method of producing a colored photographic image in a gelatino-silver halide emulsion layer, which comprises exposing it and developing it with an aromatic amino developing agent containing a primary amino group in the presence of an  $\alpha$ -naphthol containing at least one sulphonamide group.

9. A photographic emulsion for forming colored images comprising a carrier containing a

sensitive silver halide and a coupler compound selected from the group consisting of phenols and naphthols containing at least one sulphonamide group.

10. A photographic emulsion for forming colored images comprising a carrier containing a sensitive silver halide and a coupler compound comprising an  $\alpha$ -naphthol containing at least one sulphonamide group.

11. A color-forming photographic layer com- 10

prising a gelatino-silver halide emulsion containing a coupler compound selected from the group consisting of phenols and naphthols containing at least one sulphonamide group.

5 12. A color-forming photographic layer comprising a gelatino-silver halide emulsion containing a coupler compound comprising an  $\alpha$ -naphthol containing at least one sulphonamide group.

KARL SCHINZEL.